



US008262814B2

(12) **United States Patent**  
**Zak**

(10) **Patent No.:** **US 8,262,814 B2**  
(45) **Date of Patent:** **Sep. 11, 2012**

(54) **COMPOSITE ARTICLE AND METHOD**

(76) Inventor: **Gad Zak**, Pointe-Claire (CA)

(\*) Notice: Subject to any disclaimer, the term of this patent is extended or adjusted under 35 U.S.C. 154(b) by 674 days.

(21) Appl. No.: **12/272,675**

(22) Filed: **Nov. 17, 2008**

(65) **Prior Publication Data**

US 2009/0199932 A1 Aug. 13, 2009

(30) **Foreign Application Priority Data**

Nov. 15, 2007 (CA) ..... 2310534

(51) **Int. Cl.**

**C23C 8/10** (2006.01)

**C22F 1/18** (2006.01)

(52) **U.S. Cl.** ..... **148/281**; 148/669; 148/672

(58) **Field of Classification Search** ..... 148/281, 148/421, 669-672; 420/417, 422

See application file for complete search history.

(56) **References Cited**

U.S. PATENT DOCUMENTS

5,037,438 A 8/1991 Davidson

5,169,597 A 12/1992 Davidson

5,868,879 A \* 2/1999 Amick et al. ..... 148/669  
6,093,259 A 7/2000 Watanabe et al.  
6,447,550 B1 \* 9/2002 Hunter et al. ..... 623/22.15  
6,759,134 B1 7/2004 Rosenberg

FOREIGN PATENT DOCUMENTS

GB 1305879 \* 2/1973

OTHER PUBLICATIONS

Yoshiaki Ikarashi: "Improved Biocompatibility of Titanium-Zirconium (Ti-Zr) Alloy: Tissue Reaction and Sensitization to Ti-Zr Alloy Compared with Pure Ti and Zr in Rat Implantation", Oct. 13, 2006, Tokyo Dental and Medical University.

\* cited by examiner

*Primary Examiner* — Stanley Silverman

*Assistant Examiner* — Brian Walck

(74) *Attorney, Agent, or Firm* — Defillo & Associates, Inc; Evelyn A. Defilló

(57) **ABSTRACT**

Method, and articles therefrom, for providing a hard, abrasion-resistant, attractive, oxide surface layer of selectable thickness and having an outer appearance within the scale from gray to blackness, to a zirconium titanium alloy article by heating the article in an oxygen containing atmosphere.

**9 Claims, 1 Drawing Sheet**





**1**  
**COMPOSITE ARTICLE AND METHOD**

**FIELD**

The present invention relates to methods for forming a protective dark oxide layer or coating upon an article comprising zirconium, and to articles formed thereby. More specifically, the invention relates to the formation of a protective dark oxide layer upon an article consisting of certain binary zirconium titanium alloys, and to the articles formed thereby.

**BACKGROUND**

With the increase in civil use of what was considered during the "cold war" years "strategic" or "restricted" metals, such as zirconium and titanium, and the accompanying drop in their prices, an increasing number of consumer goods, medical, dental and orthopedic, civil engineering and architectural structural and decorative components, and other industrial as well as civil and military uses have been made of metals such as zirconium, titanium, and alloys thereof. With this increase in use, there has been a growing interest in their unique metallurgical properties and advantages as employed in known and new applications. These properties include very high tensile and yield strength, light weight, and chemical inertness together with its corollary hypoallergenic property, which makes these metals and alloys suitable for dental, orthopedic and other prostheses such as joint replacements, arterial stents, and cardiac valves, as well as for consumer fashion accessories that benefit from the same properties, such as body-piercings, wrist watches, sunglass frames, and the like.

Increased interest in these metals and their uses has been accompanied by demand for methods for providing hardened surfaces, for providing surfaces exhibiting reduced friction, and for improving surface appearance. At the same time, their strength, low elasticity and ductility has rendered them materials of choice for stealth activities, from hunting to law enforcement and the military, for which dark colors are preferred.

Anodizing is known for altering the color and surface appearance of titanium and niobium. Anodizing of these metals and certain of their alloys generates a thin, colorful outer layer on the metal, which wears off readily and is easily scratched, chipped, or otherwise removed.

U.S. Pat. No. 6,093,259 to Watanabe et al. teaches methods for providing various colored surfaces on titanium by treatment with aqueous alkaline solutions of KOH, NaOH and LiOH, applied singly or as a mixture, optionally accompanied by thermal treatment at moderate temperatures, and optionally comprising a nitriding process.

U.S. Pat. No. 5,037,438 to Davidson, and U.S. Pat. No. 5,169,597 to Davidson et al., disclose surface treatment of another cold war metal, zirconium, by thermal or salt bath oxidation within temperature ranges readily achievable by conventional kilns, for improving mechanical and metallurgical properties. The resulting smooth and very hard blackened surface reportedly reduced friction, increased scratch resistance, enhanced the strength of the metal immediately beneath the surface coating, and provided a blue/blackness colored surface. These enhancements were attributed to oxygen diffusion into the substrate metal, which also improved the fatigue properties of the metal.

In attempting to produce articles that require or would benefit from the combination of high tensile strength, hardness, scratch and wear resistance, and color control from dark

gray to blackness, light weight, and hypoallergenicity, it is known that zirconium and titanium provide these benefits to varying degrees.

However, unalloyed titanium colored according to the method taught by Watanabe et al. does not exhibit enhanced resistance to wear and generally retains the properties of untreated titanium. Also, the method requires the use of hazardous materials, personal safety equipment such as gas masks, impermeable gloves, complete skin coverage, and the like.

Using unalloyed zirconium to the extent taught by Davidson, is limited to unalloyed zirconium or alloys containing at least 80% zirconium, and preferably from about 95% to about 100%, by weight. In contrast, Davidson et al. teach the use of a ternary alloy including niobium, adding cost and complexity compared to binary alloys. Davidson and Davidson et al. are primarily directed to weight bearing prosthetic implants, for which color control is relatively unimportant.

While unalloyed zirconium displays high tensile strength, hypoallergenicity, and a beneficial surface coating when oxidized, it is known that alloys containing both zirconium and titanium offer superior metallurgical properties compared to each metal alone. Yoshiaki, I. et al. "Improved Biocompatibility of Titanium-Zirconium (Ti—Zr) Alloy: Tissue Reaction and Sensitization to Ti—Zr Alloy Compared with Pure Ti and Zr in Rat Implantation" Mater. Trans. 46(10): 2260-2267 (2005) (teaching superior biocompatibility of Ti—Zr alloys compared to each metal alone).

Certain ratio ranges of zirconium to titanium exhibit superior mechanical properties compared to the component metals in the unalloyed state. Kobayashi, E. "Mechanical properties of the binary titanium-zirconium alloys and their properties for biomedical purposes" J. Biomed Materials Research 29(8) (1995). Alloys in the range of 1:1 zirconium: titanium by weight, disclosed for use as dental implants, exhibit hardness and tensile strength about 2.5 times as high as the unalloyed components. These results were reported for both cast and homogenized specimens.

Ternary alloys containing zirconium, titanium and a third metal are also known for applications including prostheses. U.S. Pat. No. 5,820,707 and to Amick et al. teach ternary alloys including a third metal selected from niobium, tantalum and vanadium. The third metal is taught as passivating the tendency of the zirconium and titanium to ignite and combust. Amick et al. teaches very high temperatures and long duration for complete or near complete oxidation of the alloy workpiece, which therefore requires passivation through the inclusion of the third metal in the alloy. The method reportedly provides smooth and hard surfaces, which for some alloys are described as being "blue/blackness".

U.S. Pat. No. 6,759,134 to Rosenberg discloses ternary alloys containing titanium, niobium, and a third metal from the group consisting of zirconium, tantalum, molybdenum, hafnium, zirconium, chromium, with emphasis on alloys containing from 3% to 17% by weight niobium for its passivating properties and for the creation of a smooth and hard surface layer of niobium containing oxide with an aesthetic chromatic value.

However, Amick et al. and Rosenberg require at least a ternary alloy, do not teach control of the surface shade on a scale from dark gray to blackness, and do not teach the benefits of enhanced tensile strength of the treated alloy.

In sum, Yoshiaki et al. and Kobayashi et al. teach binary zirconium titanium alloys of specified weight ratio that possess good metallurgical, mechanical and hypoallergenic properties. The ternary alloys of Amick et al. and Rosenberg are more intricate and costly to produce and have not been

shown to possess the additional strength and hypoallergenic benefits of the binary alloy. Davidson and Davidson et al. teach the benefits of zirconium based alloys comprising a zirconium oxide coating, while Rosenberg and Amick et al. offer combinations that rely upon the presence of niobium oxide in the coating, which form of the oxide was not shown to possess the same enhanced strength and fatigue resistance as the primarily zirconium oxide coating disclosed by Davidson.

While the prior art provides a subset of the group of properties required by and benefiting various articles, namely, high tensile strength, high hardness, low ductility and elasticity, enhanced fatigue resistance, and biocompatibility, it does not teach the capability to combine the full scope of all of these benefits, the advantages in the capability to have controllable shades of dark gray to black and nor does it offer the benefits of simplicity and cost reduction to be gained through the use of a binary alloy.

Therefore, there is a need in the art for alloys and surface coatings capable of providing articles exhibiting all of the potential beneficial properties available from zirconium titanium binary alloys. All this and more will become apparent to one of ordinary skill upon reading the following disclosure and claims.

## SUMMARY

The present invention is directed in one aspect to a method for overcoming the aforementioned disadvantages and limitations of the prior art by providing a method for darkening and hardening the surface of an article consisting of a binary zirconium titanium alloy of specified composition. The inventor has found a synergistic combination, within articles produced by the method, of the metallurgical, mechanical, and hypoallergenic advantages of certain binary zirconium titanium alloys, combined with a hardened, darkened surface that resists abrasion, and has a color from gray to blackness that is selectable according to the parameters of the method.

In a first aspect, a method having features of the present invention includes the a step of providing an article consisting of between about 30.9% and about 65.6% zirconium by atomic weight and titanium. Without limitation, the articles can be formed into their desired shapes by machining, casting, die forging, stamping, or the like. The articles optionally comprise a polished, satin, or matte finish, which influences the texture of the finished blackened surface. The method further comprises heating the article in an oxygen containing atmosphere at a temperature of between about 250 and about 880 degrees Celsius for between about 10 and about 110 minutes to produce the hardened, darkened surface. In certain preferred aspects the alloy consists of between about 34.4% and about 65.6% zirconium by atomic weight.

In a second aspect, a method having features of the present invention includes the a step of providing an article consisting of between about 18.4% and about 30.9% zirconium by atomic weight and titanium. The method further comprises heating the article in an oxygen containing atmosphere in a first heating step and a second heating step with a quenching step interposed, the heating steps being performed at a temperature of between about 250 and about 880 degrees Celsius for a total duration of between about 10 and about 110 minutes to produce the hardened, darkened surface. Optionally, the first heating step is performed at a lower temperature than said second heating step. For example, and without limitation, in certain embodiments, the first heating step is carried out at a temperature of between about 250 and about 480 degrees Celsius for between about 10 and about 40 minutes,

and the second heating step is carried out at a temperature of between about 480 and about 880 degrees Celsius for between about 10 and about 70 minutes.

In certain embodiments, the oxygen containing atmosphere is air.

In another aspect, an article having features according to the present invention comprises zirconium titanium binary alloy article consisting of between about 30.9% and about 65.6% zirconium by atomic weight and titanium further comprising a darkened oxide containing surface or portion thereof produced according to one of the foregoing methods.

In certain preferred aspects the article consists of between about 34.4% and about 65.6% zirconium by atomic weight.

In another aspect, an article having features according to the present invention comprises zirconium titanium binary alloy article consisting of between about 18.4% and about 30.9% zirconium by atomic weight and titanium further comprising a darkened oxide containing surface or portion thereof produced according to one of the foregoing methods.

It is therefore an object of the present invention to provide articles that require or benefit from any combination of properties from within the group comprising, without limitation, high tensile strength, high hardness, resistance to fatigue or wear or scratch, low ductility and elasticity, hypoallergenicity, and shades of gray and blackness.

It is a further object of the invention to provide articles comprising an aesthetic outer surface or coating that exhibits shades from gray to blackness.

It is a further object of the invention to provide articles comprising a darkened surface suitable for stealth goods, hunting and sporting equipment, and body adornments that are night stealthy such as a soldier's bracelet or ring.

It is a further object of the invention to provide a ceramic-like coating that exhibits low wear and low friction suitable for articles requiring extended periods of mechanical contact, such as for example butterfly valves.

It is a further object of the invention to provide a matte or satin coating that has low reflectivity and is suitable for night-time stealth articles.

These and other features, aspects, and advantages of the present invention will become better understood with reference to the following description and appended claims.

## BRIEF DESCRIPTION OF THE DRAWING

FIG. 1 shows a cross-section of an article according to the present invention.

## DESCRIPTION

The composition of binary zirconium titanium alloys in the present disclosure are expressed by atomic weight ratio, in part to draw attention to the possibility of using unalloyed titanium and zirconium in preparing the alloys according to the present invention, despite the market's offerings of various popular alloys of titanium and zirconium. To convert from atomic weight ratio to actual weight ratio, the product of a selected element's atomic weight and its atomic weight ratio in percentage is divided by the sum of such products for the alloy constituents. For example, a ratio of 34.42% zirconium to 65.58% titanium by atomic weight, given an atomic weight for Ti of 47.867 and an atomic weight for Zr as 91.224, provides the following for the titanium ratio by weight:

$$\frac{47.867 \times 65.58\%}{(47.867 \times 65.58\% + 91.224 \times 34.42\%)} \times 100 = 49.99\%$$

the balance zirconium, or art-recognized levels of impurities.

The binary zirconium titanium alloys for use in the methods and articles according to the present invention consist of between about 18.4% and about 65.6% zirconium by atomic weight and titanium. Trace amounts of impurities, including other metals, may be present to an art-recognized degree. Certain alloys for use in the present invention can be purchased from any of several metal alloy-producing mills producing zirconium titanium alloys worldwide, and in particular in North America, and in Central and Eastern Europe.

In preferred embodiments, a binary alloy consisting of from about 65.58% titanium by atomic weight (about 50% by weight) and about 34.42% zirconium by atomic weight (about 50% by weight) is used, or alloys are used that fall within about 4% of these values. Kobayashi et al. (supra) report superior strength and hardness, up to 2.5 fold, of these alloys compared to pure zirconium and titanium.

The articles of the present invention can be made by any means known in the art for shaping zirconium titanium alloys, including without limitation machining, casting, stamping, or die-forging. It is known that certain compositions of zirconium titanium alloys are ignitable (see, e.g. U.S. Pat. No. 5,820,707 to Amick et al.) and highly reactive so due care must be taken when working such alloys. Machining requires precautionary measure as are known in the art, including but not limited to slow speeds and liberal lubrication and cooling. Likewise, opening of a casting investment must be performed only after complete cooling.

The article is heated, preferably by heating in a kiln providing an oxygen containing ambient gas, to within the range of about 250 degrees Celsius to about 880 degrees Celsius. In certain embodiments, a single heating step is provided comprising a duration of from about 10 to about 110 minutes, followed by air cooling, water quenching, or the like.

The inventor has found that with an increased gas supply, oxidation proceeds more rapidly but is accompanied by an increased risk of combustion. In preferred embodiments, a kiln is selected to have a moderate and unforced air supply in the range of 4 to 6 square inches per cubic foot of kiln volume.

Preferably, two heating steps are used, with a quenching step such as a water or air quenching interposed between the heating steps. The temperature and duration of heating are selected to provide a strongly adherent oxide-rich layer with the desired shade from gray to blackness and sufficient wear resistance. Outer layers or coatings having a darker appearance exhibit excellent resistance to wear and penetrate somewhat deeper into the substrate alloy. Where the surface of the article to be treated is polished, a smooth coating is obtained that is sufficiently hard and wear resistant to be particularly suited for uses involving frequent sliding contact with other surfaces, or impacts, or the like. Articles to be treated that have a brushed surface texture provide lighter shades.

Referring now to FIG. 1, there is shown an article according to the present invention comprising a zirconium titanium alloy **100** and a darkened surface **102**.

Most preferably, a first heating step at a lower temperature is followed by a second heating step, with a quenching step interposed between the two. This process has been found beneficial to reduce ignition risk. In preferred embodiments, a first heating step can comprise heating to between about 250 degrees Celsius to about 480 degrees Celsius for between about 10 to about 40 minutes. Following an optional quenching step, a second heating step can be performed by heating to between about 480 degrees Celsius to about 880 degrees Celsius for up to about 100 minutes or until a predetermined gray tone or degree of blackness is obtained.

Not to be thereby limited by theory, the thermal treatment of the present invention provides an oxide layer that is

believed to comprise a high proportion of zirconium oxide and to further harden and strengthen the metal by the diffusion of oxygen within the partially oxidized surface layer, and in the deeper alloy substrate to which it is adherent. In 5 embodiments comprising two heating steps, it is believed that a thicker final oxide layer is formed due to the possibility that oxygen penetrates more deeply into the substrate metal during a first, lower temperature, step than it does if exposed to an initial higher temperature that produces a more rapid thickening of the oxide layer.

Articles treated according to the method of the present invention are less susceptible to subsequent ignition. Exposure of treated samples to direct flame in the range of 1,300 to 1,400 degrees Celsius for up to ten minutes failed to combust or undergo further oxidation. This property usefully extends the range of applications of the present invention to include, for example, firearm parts, subject to proper testing and certification.

## EXAMPLES

Alloys for use in the method and article of the present invention are exemplified in TABLE 1:

| ALLOY | % Zr by atomic wt. | % Ti by atomic wt. |
|-------|--------------------|--------------------|
| I     | 34.42              | 65.58              |
| II    | 33.52              | 66.48              |
| III   | 30.89              | 69.11              |
| IV    | 40.05              | 59.95              |
| V     | 67.37              | 32.63              |

In TABLE 2, it is demonstrated that the duration and temperature of thermal treatment can be adjusted to control the resulting shade of gray or blackness in the resulting article. A darker surface is obtained with longer and/or hotter treatment, while a lighter gray finish is obtained at lower temperatures and/or shorter duration.

Results obtained with the present invention are compared in TABLE 2 with unalloyed zirconium (Zr702) and a zirconium alloy with low levels (2-3%) of niobium (Zr705).

TABLE 2

| Formation of a darkened, hardened coating according to the method of the present invention. |       |                 |                |                 |                |                               |
|---------------------------------------------------------------------------------------------|-------|-----------------|----------------|-----------------|----------------|-------------------------------|
|                                                                                             | Alloy | 1st cycle (min) | 1st cycle (C.) | 2nd cycle (min) | 2nd cycle (C.) | Resulting surface*            |
| 45                                                                                          | 1 II  | 25              | 250            | 50              | 750            | Dark blackness, smooth*       |
| 50                                                                                          | 2 VI  | 35              | 250            | 35              | 680            | Medium blackness, smooth*     |
| 55                                                                                          | 3 II  | 30              | 350            | 30              | 725            | Pitch blackness, smooth*      |
| 60                                                                                          | 4 VI  | 40              | 650            | —               | —              | Light blackness, smooth*      |
| 65                                                                                          | 5 II  | 65              | 600            | —               | —              | Medium blackness, matte       |
|                                                                                             | 6 VI  | 30              | 250            | 80              | 480            | Medium gray, smooth*          |
|                                                                                             | 7 II  | 25              | 650            | —               | —              | Medium charcoal gray, smooth* |

TABLE 2-continued

| Formation of a darkened, hardened coating according to the method of the present invention. |                 |                |                 |                |                                        |  |
|---------------------------------------------------------------------------------------------|-----------------|----------------|-----------------|----------------|----------------------------------------|--|
| Alloy                                                                                       | 1st cycle (min) | 1st cycle (C.) | 2nd cycle (min) | 2nd cycle (C.) | Resulting surface*                     |  |
| 8 VI                                                                                        | 13              | 880            | —               | —              | Light to medium charcoal gray, smooth* |  |
| 9 II                                                                                        | 11              | 880            | —               | —              | Light to medium gray, smooth*          |  |
| 10 Zr702                                                                                    | 35              | 620            | —               | —              | Medium charcoal, matte                 |  |
| 11 Zr702                                                                                    | 70              | 700            | —               | —              | Pitch blackness, smooth*               |  |
| 12 Zr705                                                                                    | 40              | 650            | —               | —              | Light charcoal, matte                  |  |
| 13 Zr702                                                                                    | 25              | 300            | 26              | 600            | Medium to dark charcoal, matte         |  |

\*articles polished prior to treatment

In a further example, a night-stealth automotive and/or stealth automotive hubcap is provided. The hubcap is cast into the desired shape and provided with a satin-like low-polish. The hubcap is then heated to within the range of 250 to 350 degrees for from 10 to 40 minutes. Next, the hubcap is heated by the same method for 20 to 40 minutes at 600 to 700 degrees Celsius. The hubcap is from charcoal gray to blackness in appearance and has a matte, wear resistant surface.

In use, the method of the present invention is used to produce articles that are also encompassed by the present invention. The articles can be any article consisting of zirconium titanium alloy within the composition range of the present invention that requires or may benefit from a hard, tough, gray to blackness outer surface layer. Without limitation, articles within the scope of the present invention can include articles that comprise pivoting or swiveling parts such as revolving disk and butterfly valves, cardiac valves, and valves for liquids and gases. In these applications, the swiveling parts can be springingly retained about their axis by insertion under tensile stress between mounting points, or more loosely retained. Other article embodiments can include dental implants and medical prostheses such as joint and bone replacements. Further, the present invention can provide a tough and attractive outer surface to sporting goods such as golf clubs, durable and night-stealth hunting goods such as knives, outdoors equipment such as binocular outer casings, bow coatings, water canteens, field-compasses and the like. The articles according to the present invention can be stealth items such as for law enforcement and armed forces, such as helmets, buckles, ID tags, night vision equipment, laptop and communications and data storage equipment casings, firearms and parts thereof such as sights, triggers, cartridges, magazines, barrels, and the like. Other articles within the scope of the present invention are night-stealth compatible jewelry items of low wear, for use by armed forces and law enforcement personnel, for example bands including bands that benefit from the invention's metallurgical attributes of excellent strength, tensile strength, low elasticity and ductility, and therefore, strong springiness, wherein a stone may be set under pressure and retained between two connected por-

tions of the band. Such stealth compatible and low wear jewelry items can further comprise wedding bands, buckles, bracelets, chains, earrings, watches, chains, sunglass frames, cuff links, tie-pins, money or document clips, bracelets and necklaces. The darkened surface of jewelry according to the present invention can provide an aesthetic and/or a utilitarian function. Yet further, marine and/or night-stealth marine items such as boat masts, deck handles, steering wheels, throttles; automotive and/or stealth automotive parts such as gearshift levers, hubcaps, steering wheels; and household items such as door handles, cabinet handles, keys, cutlery, faucets, light fixtures and kitchen implements can all be provided within the scope of the present invention. Yet further examples can include musical instruments, such as brass instruments with valves, for which the hypoallergenic and excellent wear resisting properties of the instant invention are well suited. Still further example include architectural structural and surface materials, for which a darkened surface prepared according to the method of the present invention can be used to alter the structural and surface material thermal properties and the lightness of the alloy may also be beneficial.

This invention has been described with respect to its preferred embodiments and contemplated utility. Variations can be made without undue experimentation by those skilled in the art with the expected results being obtained without departing from the spirit and scope of the invention described in the appended claims as interpreted in view of the applicable prior art.

What is claimed is:

1. A method for producing an article having a darkened surface, the method consisting of the steps of:
  - providing an article made from an alloy consisting of between about 18.4% and about 65.6% of zirconium by atomic weight and titanium;
  - heating the article in an oxygen containing atmosphere at a temperature of between about 250 and about 880 degrees Celsius for a period between about 10 and about 110 minutes;
  - the heating step includes a first heating step, a quenching step following the first heating step, and a second heating step.
2. The method of claim 1, in which said first heating step is performed at a lower temperature than said second heating step.
3. The method of claim 2, in which the first heating step is carried out at a temperature of between about 250 and about 480 degrees Celsius for between about 10 and about 40 minutes.
4. The method of claim 2, in which the second heating step is carried out at a temperature of between about 480 and about 880 degrees Celsius for between about 10 and about 70 minutes.
5. The method of claim 1, in which the alloy contains between about 34.4% and about 65.6% zirconium by atomic weight.
6. The method according to claim 1, in which said oxygen containing atmosphere is air.
7. The method according to claim 1, in which the article is a machined, cast, or die-forged article.
8. The method according to claim 1, wherein the darkened surface has a matte or satin finish.
9. The method according to claim 1, wherein the darkened surface includes a gray black color.